

## UNITED STATES PATENT OFFICE.

HOWARD WATERS DOUGHTY, OF AMHERST, MASSACHUSETTS, ASSIGNOR TO ALCHEMIC GOLD COMPANY, INC., A CORPORATION OF NEW YORK.

## INK.

No Drawing.

Application filed May 8, 1922. Serial No. 559,419.

To all whom it may concern:

Be it known that I, HOWARD WATERS DOUGHTY, a citizen of the United States, residing at Amherst, in the county of Hampshire, State of Massachusetts, have invented certain new and useful Improvements in Inks; and I do hereby declare the following to be a full, clear, and exact description of the invention, such as will enable others skilled in the art to which it appertains to make and use the same.

This invention relates to inks and vehicles therefor, and particularly to metallic pigment inks suitable for use in stamping titles and decorative designs on book bindings and for other purposes to which the ink may be adapted.

In stamping titles in gold, for example, on books, labels and like materials, it has been the practice heretofore to employ gold or imitation gold leaf. The leaf is applied manually after the surface of the material has been treated with size, and the surplus leaf must be removed after stamping. Several operations are thus involved and the application of leaf in the manner described is consequently expensive. The use of artificial leaf effects a saving only in the cost of the leaf. Artificial leaf is, moreover, unsatisfactory because of the inferior quality of the work which quickly tarnishes when exposed to the effect of the atmosphere.

The use of metallic pigment inks has been suggested heretofore as a substitute for metallic leaf in stamping operations. No suitable inks have been available, however, and it has been impossible to produce satisfactory work therewith. A difficulty which has prevented the use of metallic pigment inks is due to vehicles which dry too rapidly on the inking rolls, covering them generally with a gummy coating which prevents transfer of the ink to the type or die. In avoiding this extreme it is necessary to provide an ink which when once applied will dry rapidly.

It is the object of the invention, therefore, to provide an ink and an ink vehicle having the necessary properties, among others comparative slowness in drying without a tendency to become gummy, a consistency permitting transference of the ink through

inking rolls to the type or die, rapid drying when applied to the work, and ability to protect the pigment from oxidation and consequent discoloration.

I have discovered that these desirable properties may be imparted to the ink by the use of a suitable medium in the vehicle for the pigment and that such a medium will, moreover, permit rapid drying of the ink by the application of heat to the type or die. The medium should be volatile, i. e., capable of being vaporized without carbonization, but its boiling point should be relatively high to reduce vaporization at atmospheric temperatures, and consequently to prevent rapid drying on the inking rolls. The medium must, moreover, be a solvent for the body of the vehicle. Preferably the boiling point of the selected medium should be between 200° and 300° C., a boiling point lower than 250° C. being desirable. Solvents boiling materially below 200° C. are unsuitable because the ink dries too rapidly on the rolls and becomes gummy. Solvents boiling materially above 300° C. are likewise unsuitable because the ink cannot be successfully dried except by the application of impractically high temperatures. A suitable medium may be found in the derivatives of the terpene series of hydrocarbon compounds, the alcohols, of which terpineol is an example, being admirably adapted for the purpose. Terpineol is capable of imparting the desired properties to the vehicle in a marked degree, and is at the same time readily available in commerce and relatively inexpensive. Other suitable solvents are benzyl alcohol and certain esters of aromatic acids such as terpinyl acetate, benzyl acetate and ethyl benzoate. Oil of dammar resin is also a suitable solvent, this and the other solvents mentioned having the distinguishing characteristics above referred to.

In carrying out the invention the solvent is combined with a thickening agent forming the body of the vehicle. Preferably a resinous material such as colophony (ordinary rosin), dammar, copal, Burgundy pitch or Canada balsam, is dissolved in the solvent to produce a vehicle of the desired consistency. A proportion of benzoin may be added with advantage to the composition, replacing a

portion of the other resinous material, or benzoin may be substituted for either of the resins mentioned, which, of course, may be mixed or combined in any desired proportions, although for commercial reasons it is preferred to employ colophony alone as a resinous ingredient of the composition. The pigment, preferably a bronze or other metallic powder of the desired color, is thoroughly 5 incorporated with the vehicle to complete the ink.

It is to be understood that equivalents of the terpineol, benzyl alcohol or other solvent may be substituted therefor and that 10 materials naturally containing these solvents may be employed. Artificial mixtures containing the solvents mentioned may be used also. Natural or artificial mixtures of the solvent should have a minimum 15 boiling point of substantially 200° C. to avoid too rapid drying of the ink upon the rolls.

The bronze or other metallic powder used may be the ordinary article of commerce 20 and may consist, for example, of an alloy of copper with other metal or metals adapted to impart the desired color to the alloy. The alloy is reduced to a state of fine subdivision in the usual manner. Metallic 25 powders containing metals other than copper can be used.

As an example of the application of the invention, the vehicle may comprise four 30 parts of the solvent, benzyl alcohol for example, to one part of ordinary rosin. Preferably the benzyl alcohol is heated to a temperature ranging from 100° to 130° C. and is maintained at that temperature while the rosin is dissolved therein. The proportions 35 of resin and solvent may be varied within the limits necessary to produce a vehicle of the proper viscosity. The vehicle and metallic powder are thoroughly mixed preferably in the proportions of two parts 40 of the powder to one part of the vehicle.

The ink produced as described may be applied by means of the usual ink fountain or 45 table to the inking rollers and thence transferred to the type or die. Drying of the ink on the rollers, a fault which has characterized inks heretofore suggested, is 50 avoided. The ink dries very slowly at atmospheric temperature owing to the high 55 boiling point of the volatile solvent. It dries rapidly, however, when applied with a heated die. The impression is highly 60 glossed and the vehicle forms a lacquer which protects the pigment from tarnishing, thus providing a permanent and highly 65 satisfactory title or decoration on book bindings and the like. The color will depend upon the particular pigment employed which may be other than metallic in character.

65 The ink described, though particularly

suitable for book-binders' use, will serve other purposes of decorative printing. It is adapted to materially reduce the cost of such printing because of the low cost of the ink and the simplicity of its application.

70 Various changes may be made in the details of the invention without departing therefrom or sacrificing any of the advantages thereof.

I claim:

1. An ink having a metallic pigment and a vehicle comprising a resinous substance and a volatile solvent therefor, the boiling point of which is not materially lower than 200° C.

75 2. An ink having a metallic pigment and a vehicle comprising a resinous substance and a volatile solvent therefor with a boiling point between 200° and 300° C.

3. An ink having a metallic pigment and a vehicle comprising a resinous substance and a volatile solvent therefor with a boiling point between 200° and 250° C.

80 4. An ink having a metallic pigment and a vehicle comprising ordinary rosin and a volatile solvent therefor, the boiling point of which is not materially lower than 200° C.

5. An ink having a metallic pigment and a vehicle comprising ordinary rosin and a volatile solvent therefor with a boiling point 85 between 200° and 300° C.

6. An ink having a metallic pigment and a vehicle comprising ordinary rosin and a volatile solvent therefor with a boiling point 90 between 200° and 250° C.

7. An ink having a metallic pigment and a vehicle comprising a resinous substance and benzyl alcohol as a solvent therefor.

105 8. An ink having a metallic pigment and a vehicle comprising a resinous substance and a solvent therefor containing benzyl alcohol.

9. An ink having a metallic pigment and a vehicle comprising a solvent containing 110 benzyl alcohol and a thickening agent dissolved therein.

10. An ink having a metallic pigment and a vehicle comprising a solvent, the boiling point of which is not materially lower than 115 200° C. and a thickening agent dissolved therein.

11. An ink having a metallic pigment and a vehicle comprising a solvent with a boiling point between 200° and 300° C. and a thickening agent dissolved therein.

12. An ink having a metallic pigment and a vehicle comprising a solvent with a boiling point between 200° and 250° C. and a thickening agent dissolved therein.

13. In an ink a vehicle comprising a resinous substance and a volatile solvent therefor, the boiling point of which is not materially lower than 200° C.

130 14. In an ink a vehicle comprising a

- resinous substance and a volatile solvent therefor with a boiling point between 200° and 300° C.
15. In an ink a vehicle comprising a resinous substance and a volatile solvent therefor with a boiling point between 200° and 250° C.
16. In an ink a vehicle comprising ordinary rosin and a volatile solvent therefor, the boiling point of which is not materially lower than 200° C.
- 10 17. In an ink a vehicle comprising a resinous substance and benzyl alcohol as a solvent therefor.
- 15 18. In an ink a vehicle comprising a resinous substance and a solvent therefor containing benzyl alcohol.
19. In an ink a vehicle comprising a solvent containing benzyl alcohol and a thickening agent dissolved therein.
- 20
20. In an ink a vehicle comprising a solvent containing benzyl alcohol and ordinary rosin dissolved therein.
21. In an ink a vehicle comprising ordinary rosin and benzyl alcohol as a solvent therefor.
22. In an ink a vehicle comprising a solvent, the boiling point of which is not materially lower than 200° C. and a thickening agent dissolved therein.
23. In an ink a vehicle comprising a solvent with a boiling point between 200° and 300° C. and a thickening agent dissolved therein.
24. In an ink a vehicle comprising a solvent with a boiling point between 200° and 250° C. and a thickening agent dissolved therein.

In testimony whereof I affix my signature.  
HOWARD WATERS DOUGHTY.